

# UNITED STATES PATENT OFFICE.

AUGUSTUS SCHULTZ, OF NEW YORK, N. Y.

## TAWING HIDES AND SKINS.

SPECIFICATION forming part of Letters Patent No. 291,784, dated January 8, 1884.

Application filed May 31, 1883. (No specimens.)

*To all whom it may concern:*

Be it known that I, AUGUSTUS SCHULTZ, a citizen of the United States, residing at New York, in the county and State of New York, 5 have invented a new Improved Process of Tawing Hides and Skins, of which the following is a specification.

This invention relates to a new process for tawing hides or skins, said process consisting 10 in subjecting said hides or skins to the action of compounds of metallic salts—such as bichromate of potash—and then treating the same with hyposulphite of soda, by which term is understood that salt which is more recently 15 sometimes called "thiosulphate of soda," ( $\text{Na}_2\text{S}_2\text{O}_3$ ).

In carrying out my process, I unhair the rawhides and prepare them in the same manner in which they are made "ready" for tanning. 20 If the hides have not been pickled, I subject them to the action of a solution of bichromate of potash in the presence of an acid—such as hydrochloric acid—or, if the hides have been pickled, they may be treated 25 in a solution of bichromate of potash in water without the addition of an acid. In this solution the hides are left for a shorter or longer time, according to their thickness and to the strength of the solution employed. A skiver 30 or the face of a sheep-skin can be done in a strong solution, as above described, in about fifteen minutes, while a full skin "roan" would require in the same solution about one hour. I call the solution "weak" if it contains 35 five per cent. or less of the weight of skins of bichromate of potash, and I call the solution "strong" if it contains more than five per cent. of bichromate of potash. It is not material, however, how strong the solution is. 40 The skins are completed if small pieces cut from the thickest parts of said skin show that the solution has entirely penetrated. The skins are then ready to be taken out, and after the adhering liquor has run off the skins 45 are introduced into the second solution, which consists of hyposulphite of soda dissolved in water, and adding an acid, such as hydrochloric acid. The solution may be strong or weak of hyposulphite, and the quantity of 50 acid used at first may be less than requisite to split up the entire quantity of hyposul-

phite, and more acid may be added if the skins show that more is required, which is indicated by the color of the skins. When they are done, they show a whitish, blueish, 55 or greenish color, according to the time they are kept in the hyposulphite solution. A skiver which first has been exposed to the action of the bichromate for fifteen minutes will be ready by remaining in the hyposulphite solution about twenty minutes. For thicker skins a proportionately longer time is required. For some skins—such as calf or steers' skins—it is desirable that the same, after having been withdrawn from the second 60 or hydrosulphite solution, shall be returned to the bichromate solution, which imparts to them a brownish color and leaves them in a favorable condition to be colored black. The coloring can be done after the skins leave the 65 hyposulphite solution, and after they have been exposed for the second time to the bichromate solution. The leather coming from the hyposulphite solution is especially adapted for light or dark colors, and by proper dyeing 70 methods better and brighter colors can be produced than on leather done by tanning. After the leather is treated in the manner above indicated, it may be colored, soaped, and greased in the usual way. Leather can also be made 75 by reversing the operation and first soaking the hides in a solution of hyposulphite of soda and then exposing them to the action of the bichromate solution. By using the solutions indicated at a heat of about 80° Fahrenheit, 80 the process will be done in a shorter time than if the solutions are used cold. By my process the gelatine contained in the hides is rendered insoluble by means not injurious to the leather. If leather made by tannin is put in a strong 85 soda solution, the tannin is extracted and a dark-brown liquor is formed. If leather made by my process is put in a strong soda solution, the liquor obtained shows only a little milky color. 90

Leather made by my process is very strong, 95 soft, elastic, and my process is applicable to hides or skins of every description.

What I claim as new, and desire to secure by Letters Patent, is—

The within-described process for tawing 100 hides and skins, said process consisting in sub-

jecting the hides or skins to the action of compounds of metallic salts—such as a solution of bichromate of potash—and then treating the same with a compound containing hyposulphurous acid, (or as it is otherwise called "thiosulphuric" acid,) such as a solution of hyposulphite of soda or of potash in the presence of hydrochloric acid.

In testimony whereof I have hereunto set my hand and seal in the presence of two subscribing witnesses.

AUGUSTUS SCHULTZ. [L. s.]

Witnesses:

W. HAUFF,

WILLIAM MILLER.